

## UNITED STATES PATENT OFFICE

2,512,578

METHOD OF DESULFURIZING AND  
DECOPPERIZING FERROUS METAL

James Fernando Jordan, Huntington Park, Calif.

No Drawing. Application May 26, 1949,  
Serial No. 95,591

4 Claims. (Cl. 75—53)

1

My invention relates to the desulphurization and decopperization of molten ferrous metals.

This is a continuation-in-part of my copending application Serial No. 26,937, filed on May 13, 1948, and my copending application Serial No. 49,217, filed on Sept. 14, 1948, both now abandoned.

The copper content of the steel being produced in the United States has been slowly gaining ground, as the result of the copper content of pig iron and the influx of copper-bearing metals into the steel-scrap portion of the typical steel-making charge. While a certain measure of copper is supposed to help the corrosion resistance of steel, there are other effects of copper in steel which are bad. Thus, for example, copper harms the deep-drawing properties of steel.

I have found a reagent slag that is capable of extracting copper and sulphur from molten iron or molten steel. My reagent slag contains, as its principal desulphurizing and decopperizing agent, either sodium sulphide, or potassium sulphide, or aluminium sulphide.

In my copending application, Serial No. 26,937, I disclosed my reagent slag for desulphurizing molten iron, said slag containing either sodium sulphide, or potassium sulphide, or aluminium sulphide as its principal desulphurizing agent. I have found that when sufficient sulphur is present in the ferrous metal to convert the copper content of said metal to cuprous sulphide, my previously-disclosed desulphurizing slag will also decopperize said ferrous metal.

While my discovery indicates that copper has a greater affinity for sulphur than iron has at those temperatures where ferrous metals are molten, other commonly-employed alloying constituents in said ferrous metals have a still greater affinity for sulphur. Thus, for example, manganese and aluminium both have a greater affinity for sulphur than copper has. As a consequence in the presence of such elements as said manganese and/or aluminium, copper will not combine with the sulphur content of the ferrous metal until sufficient sulphur is present to first satisfy the conversion requirements of said manganese and/or aluminium.

My practice in treating ferrous metal is to assume that the sulphur requirements of copper may be estimated by multiplying the copper content of the metal by 0.28; that the sulphur requirements of the manganese may be estimated by multiplying the manganese content of the metal by 0.64; and that the sulphur requirements of the aluminium may be estimated by multiply-

2

ing the aluminium content of the metal by 1.9. In general, the copper and manganese factors are about 10% above the assumed equation requirements; the aluminium factor being satisfactory in the presence of the usually small aluminium content of ferrous metal.

Thus, for example, in a test that I made with an iron containing 3.34% carbon, 2.10% silicon, 0.10% manganese, and 0.30% copper, I added 0.155% sulphur. Contact with molten sodium sulphide at 2500° F. lowered these values to 0.009% manganese, 0.04% copper, and 0.019% sulphur. This sodium sulphide reagent contained 20% aluminium sulphide.

In another case, I treated a molten iron containing 4.35% carbon, 3.34% silicon, 0.89% manganese, and 0.25% copper, with a 0.65% sulphur addition. Contact with a molten sodium-aluminium sulphide lowered these values to 0.05% manganese, 0.03% copper, and 0.027% sulphur.

Deoxidized steel may be treated with sulphide slag to remove copper and sulphur therefrom. In a test that I made with a steel containing 0.30% carbon, 0.41% silicon, 0.17% manganese, and 0.76% copper, I added 0.35% sulphur. Contact with molten sulphide slag containing 90% aluminium sulphide and 10% aluminium oxide lowered these values to 0.02% manganese, 0.05% copper, and 0.020% sulphur.

In another test that I made with this steel, I added enough aluminium to the steel to yield a residual aluminium content of 0.05%, and then I treated the resulting metal with 0.43% sulphur. Contact with the molten aluminium sulphide-aluminium oxide reagent gave 0.02% manganese, 0.07% copper, and 0.011% sulphur.

These molten sulphide slags must be protected from the air, for said sulphides show a marked tendency to oxidize to the corresponding sulphates. Furthermore, fume hoods are a required accessory in my process, although I have had good success in depressing the fuming of the molten sulphides by elevating their boiling points by means of the non-volatile-solute effect. Thus, I depressed the fuming of sodium sulphide by adding aluminium sulphide thereto, and I depressed the fuming of aluminium sulphide by adding aluminium oxide thereto.

If, in addition to, or in place of, manganese and/or aluminium, the ferrous metal contains other elements which have a greater affinity for sulphur than has copper, then sufficient sulphur must be added to the metal to convert these other elements into their corresponding sulphides; for, copper will not combine with sulphur in the pres-

ence of the unsatisfied demand of such other elements. Thus, for example, if the metal contains zirconium, sufficient sulphur must be added to convert said zirconium to zirconium sulphide.

Tests have shown that potassium sulphide acts in a manner similar to sodium sulphide; that is, it desulphurizes and decopperizes ferrous metal that contains its copper content as cuprous sulphide. For example, I have obtained good results with a slag composed of 60% potassium and 40% aluminum sulphide, and I have obtained good results with a slag composed of 30% potassium sulphide, 30% sodium sulphide, and 40% aluminum sulphide.

The extraction of copper from ferrous metal by my sulphide slag is apparently favored by higher extraction temperatures.

In several tests that I made, the nickel content of the molten ferrous metal was observed to have partly passed into the sulphide slag with the copper; and in certain other tests made at very low extraction temperatures, the molybdenum content of the metal passed, in part, into the sulphide slag with the copper.

The factor which I use to figure the proper concentration of sulphur in a ferrous metal to be treated for the removal of its copper content are my preferred embodiment; however, I have obtained a certain measure of decopperization with lower sulphur percentages—thus, in a test that I made with the molten iron that contained 3.34% carbon, I added 0.099% sulphur. Contact with the molten sodium sulphide-aluminum sulphide slag gave the following results: 0.009% manganese, 0.22% copper, and 0.012% sulphur.

The enumerated tests employed one pound of slag for every pound of metal treated when the sulphur content of the metal was below 0.25%, and said tests employed two pounds of slag for every pound of metal treated when the metal contained more than 0.25% sulphur.

The efficiency of my process may be greatly increased by recovering the copper-manganese-bearing waste slag. This may be done by treating said waste slag, while it is molten, with aluminum, whereupon said aluminum will displace the copper and manganese therein—yielding an alloy of copper and manganese, and aluminum sulphide.

The efficiency of the extraction may be greatly increased by employing a counter-current extractor—this in, keeping, with the well known increased efficiency derived from employing the counter-current principle in extraction processes. Counter-current extractors suitable for use in extracting sulphur and copper from molten ferrous metals are disclosed in my copending applications: Serial No. 783,391, filed on Oct. 31,

1947, now abandoned; Serial No. 69,467, filed on Jan. 6, 1949; and Serial No. 73,993, filed on Feb. 1, 1949—the latter two counter-current extractors being most suitable for use in an extraction process wherein intimate contact between the solvents and the absence of air are desirable, such as in the present case.

Having now described several forms of my invention, I wish it to be understood that my invention is not to be limited to the specific form or arrangement of steps herein disclosed, except insofar as such limitations are specified in the appended claims.

I claim as my invention:

1. The method of refining iron and steel containing copper, which comprises: melting the copper-bearing metal; adding sufficient sulphur to the molten metal to convert into their respective sulphides any metals present in said molten metal having a greater affinity for sulphur than the affinity of copper for sulphur and to convert a substantial portion of the copper present into cuprous sulphide; contacting said molten metal with a molten sulphide slag consisting essentially of a sulphide selected from the group consisting of sodium sulphide, potassium sulphide, aluminum sulphide, and mixtures thereof; and separating said slag from said metal after said molten sulphide slag has lowered the copper content of said molten metal and after said molten sulphide slag has extracted from said molten metal a substantial portion of the sulphur that was added to said molten metal.

2. The process according to claim 1 in which said molten sulphide slag consists essentially of sodium sulphide.

3. The process according to claim 1 in which said molten sulphide slag consists essentially of potassium sulphide.

4. The process according to claim 1 in which said molten sulphide slag consists essentially of aluminum sulphide.

JAMES FERNANDO JORDAN.

#### REFERENCES CITED

The following references are of record in the file of this patent:

#### UNITED STATES PATENTS

| 50 | Number    | Name      | Date          |
|----|-----------|-----------|---------------|
|    | 838,125   | Maffett   | Dec. 11, 1906 |
|    | 1,425,701 | Sem       | Aug. 15, 1922 |
|    | 1,785,503 | Spring    | Dec. 16, 1930 |
|    | 1,837,432 | Hanak     | Dec. 22, 1931 |
| 55 | 1,982,959 | Kuhlmann  | Dec. 4, 1934  |
|    | 2,109,144 | Betterton | Feb. 22, 1938 |
|    | 2,301,360 | Brennan   | Nov. 10, 1942 |